

## UNITED STATES PATENT OFFICE

1,952,459

PROCESS FOR THE RECOVERY OF  
MOLYBDENUMErnst Pokorny, Leipzig, Germany, assignor to I. G.  
Farbenindustrie Aktiengesellschaft, Frankfort-  
on-the-Main, GermanyNo Drawing. Application April 9, 1931, Serial No.  
528,983. In Germany May 2, 1930

11 Claims. (Cl. 23—22)

The present invention relates to the recovery of molybdenum from mixtures of molybdenum or its compounds, with other substances.

This invention is an improvement of the process forming the subject-matter of the application Ser. No. 478,111, filed August 27, 1930, to Karl Winkler et al., according to which molybdenum is recovered practically completely from mixtures of molybdenum or its compounds, with other metals, as for example chromium, zinc, magnesium and the like by subjecting the mixtures to a treatment with oxygen or gases containing or supplying oxygen, such as air, nitrogen oxides or the like at elevated temperatures not exceeding 600° C. and preferably below 500° C., but usually not below about 400° C. No formation of any compounds between molybdcic acid and other components of the mixture takes place, which could adversely affect the subsequent further working up of the roasted material, when carrying out the recovery in the said manner. The said subsequent treatment, for the purpose of recovering the molybdenum, may be performed by treating the roasted material with ammonia, and precipitating the molybdenum from the resulting ammoniacal solution under such conditions, as regards hydrogen-ion concentration, that complete separation of the molybdcic acid from the other constituents is obtained.

I have now found that the recovery of the molybdenum from the material roasted in the said manner is also advantageously effected by treating the latter with a solution of ammonium sulphide, which may, if necessary, contain free ammonia. The extraction of the roasted material is preferably carried out in a vessel fitted with stirrers, in which case it is advisable to employ such an amount of ammonium sulphide as will precipitate, in the form of sulphides, as much as possible of the substances accompanying the molybdenum, without causing the formation of more than a small quantity (if any) of ammonium sulphomolybdate. This amount of ammonium sulphide is equivalent to the sulphide-forming heavy metals other than molybdenum. If the amount of the sulphide-forming materials in the roasted charge is insufficient to combine with the whole of the sulphur liberated in the formation of ammonium molybdate, elements or compounds which will combine with the surplus sulphur present as sulphide ions to form insoluble sulphides are added either during or after the treatment with ammonium sulphide solution, since it is generally desirable to pre-

vent the formation of ammonium sulphomolybdate. The molybdenum, the whole of which is contained in the solution as ammonium molybdate, can be completely precipitated by acidification, for example with hydrochloric acid, the ammoniacal solution being preferably run into the acid. In so doing, it is important that a definite acidity which is generally smaller than  $n/1$ , and preferably  $n/10$ , should be maintained in order, on the one hand, to prevent the precipitated molybdcic acid from being partly redissolved, should the hydrogen-ion concentration be too high, and, on the other hand, contamination by other constituents in the event of said concentration being too low.

The advantages of extracting the roasted material with ammonium sulphide as compared with the procedure specified in the aforesaid application Ser. No. 478,111 are due to the greater solvent properties of the said sulphide, so that the extraction may be performed, for example even at ordinary temperature, and also to the smaller consumption of acid for precipitating the molybdcic acid from the ammonium molybdate solution. A further advantage consists in that the precipitation of the molybdcic acid can also be performed at ordinary temperature, because the substances forming insoluble sulphides have already been eliminated in the extraction stage.

In treating, for example, a molybdenum-zinc catalyst employed in the pressure-hydrogenation process, the zinc sulphide precipitated by the treatment with ammonium sulphide can be transformed into zinc oxide by roasting, so that not only the molybdenum, but also the zinc can be recovered, in a simple manner, in the original form present in the catalyst, whereas, in the method of operating according to the said application Ser. No. 478,111, the zinc is obtained as zinc chloride, the working up of which from the dilute solution is less economical.

The following examples will further illustrate the nature of this invention, but the invention is not restricted to these examples.

## Example 1

A catalyst employed in the pressure-hydrogenation of organic substances, and consisting of molecular proportions of molybdenum, zinc and magnesium, in the form of their oxides or sulphides, is roasted with gases containing oxygen, in the manner specified in Example 1 of the aforesaid application Ser. No. 478,111. The roasted material is then treated with a gradual addition of about 2½ litres per kilogram of a

10 per cent solution of ammonium sulphide containing about 2 per cent of free ammonia, in a vessel fitted with stirrers and at ordinary temperature, until the colour changes from light 5 yellow to orange. Under these conditions the whole of the zinc is transformed into insoluble zinc sulphide, whereas molybdenum and magnesium pass into solution, the molybdenum being entirely in the form of ammonium molybdate, free from ammonium sulphomolybdate.

10 After filtering off the insoluble zinc sulphide, the filtrate is treated, at ordinary temperature, with hydrochloric acid, in such an amount that the liquid finally contains about 0.3 per cent of 15 hydrogen chloride. Under this treatment the molybdenum is precipitated as molybdcic acid, whilst the magnesium remains in solution as chloride.

*Example 2*

20 A mass obtained by roasting a spent catalyst (see Example 1) and consisting of about 80 parts of molybdcic acid and 20 parts of zinc oxide, is treated with about 2.4 litres per kilogram of material of an ammoniacal liquor consisting of 25 0.7 litre of 10 per cent aqueous ammonia and 1.7 litres of 10 per cent ammonium sulphide solution. The amount of sulphur present in the liquid is just sufficient for the complete transformation of the zinc present into insoluble zinc sulphide, while the molybdcic acid is transformed into soluble ammonium molybdate, without formation of ammonium sulphomolybdate. The molybdcic acid can be recovered from the solution in the manner described in Example 1.

*Example 3*

40 A catalyst, roasted in the manner described in the said application Ser. No. 478,111, consisting of 80 parts of molybdcic acid, 20 parts of zinc oxide and 25 parts of magnesium oxide, is treated with an addition of a further 25 parts of zinc oxide, so as to attain the composition of the 45 roasted material mentioned in Example 1. The further treatment is performed in the manner described in that example.

45 The zinc sulphide obtained by filtering the reaction liquid is transformed into zinc oxide by roasting, and this product can then be employed in the treatment of further quantities of the specified catalyst material.

*Example 4*

50 A catalyst roasted in the manner described in the said application Ser. No. 478,111, consisting of 80 parts of molybdcic acid and 20 parts of zinc oxide is treated with about 6.2 litres per kilogram of a 10 per cent ammonium sulphide solution (containing 2 per cent of free ammonia) that the whole of the zinc is transformed into sulphide, and all the molybdenum present into ammonium sulphomolybdate.

55 The ammonium sulphomolybdate solution filtered off from the zinc sulphide is treated with sufficient zinc oxide to extract the sulphur from the sulphomolybdate and form zinc sulphide (1.8 kilograms per each kilogram of roasted catalyst). The zinc sulphide formed is converted into zinc oxide by roasting.

60 The zinc oxide may be replaced by some other compound furnishing an insoluble sulphide, such as cadmium oxide, lead oxide, stannous oxide or a mixture of several of such compounds.

*Example 5*

65 100 kilograms of a catalyst roasted in the man-

ner described in the said application Ser. No. 478,111, consisting of 90 parts of molybdcic acid and 10 parts of chromic acid, are treated with 80 630 litres of a 20 per cent aqueous solution of ammonium sulphide containing 2 per cent of free ammonia, whereby practically the whole of the molybdcic acid passed into solution as ammonium sulphomolybdate. The chromic acid remains behind undissolved. For the purpose of transforming the ammonium sulphomolybdate into ammonium molybdate, the filtered solution is treated with 560 kilograms of lead oxide. The liquid is filtered and the molybdcic acid is precipitated from the filtrate in the manner specified in Example 1. The filtration residue, consisting of lead sulphide, is transformed, by roasting, into lead oxide which can then be employed in the treatment of a further quantity of the catalyst material.

85 What I claim is:—

1. In the recovery of molybdenum from a material comprising molybdenum and at least one metal selected from the group consisting of magnesium, zinc and chromium, the steps which comprise subjecting the said material to a treatment 100 with a gas capable of liberating free oxygen at a roasting temperature not exceeding 600° C. and then converting the molybdenum oxides thus formed into soluble ammonium molybdate by treating the resulting mixture with so much of 105 a solution of ammonium sulphide in the presence of a compound having a cation capable of forming an insoluble sulphide that no substantial quantity of ammonium sulfo-molybdate remains after the conversion.

110 2. In the recovery of molybdenum from a material comprising molybdenum and at least one metal selected from the group consisting of magnesium, zinc and chromium, the steps which comprise subjecting the said material to a treatment with 115 a gas capable of liberating free oxygen at a temperature between 400 and 600° C. and then converting the molybdenum oxides thus formed into soluble ammonium molybdate by treating the resulting mixture with a solution containing ammonia and so much ammonium sulphide in the presence of so much of a compound having a cation capable of forming an insoluble sulphide that no substantial quantity of ammonium sulfo-molybdate remains after the conversion.

120 3. In the recovery of molybdenum from a material comprising molybdenum and at least one metal selected from the group consisting of magnesium, zinc and chromium, the steps which comprise subjecting the said material to a treatment 130 with a gas capable of liberating free oxygen at a temperature between 400 and 600° C., treating the resulting mixture with a solution of ammonium sulphide and adding to this solution a substance combining with the sulphide ion to form an insoluble sulphide, the amount of ammonium sulphide and said substance being so coordinated as to preclude the formation of substantial quantities of ammonium sulfo-molybdate.

135 4. In the recovery of molybdenum from a material comprising molybdenum and at least one metal selected from the group consisting of magnesium, zinc and chromium, the steps which comprise subjecting the said material to a treatment with a gas capable of liberating free oxygen at a 140 temperature between 400 and 600° C. treating the resulting mixture with a solution containing free ammonia and ammonium sulphide and adding to this solution a substance combining with the sulphide ion to form an insoluble sulphide, the 145 150

amount of ammonium sulphide and said substance being so coordinated as to preclude the formation of substantial quantities of ammonium sulfo-molybdate.

5. In the recovery of molybdenum from a material comprising molybdenum and at least one metal selected from the group consisting of magnesium, zinc and chromium, the steps which comprise subjecting the said material to a treatment with a gas capable of liberating free oxygen at a temperature ranging from 400° to 500° C. then converting the molybdenum oxides thus formed into soluble ammonium molybdate by treating the resulting mixture with so much ammonium sulphide in the presence of so much of a compound having a cation capable of forming an insoluble sulphide that no substantial quantity of ammonium sulfo-molybdate remains after the conversion.

10. The process of recovering molybdenum from a mixture containing it and at least one metal selected from the class consisting of zinc, magnesium and chromium which comprises treating the mixture with a gas capable of liberating free oxygen at a temperature ranging from 400° to 500° C. to effect a conversion of the metallic constituents of said mixture into the oxidic state, converting the oxides of molybdenum in said mixture into ammonium molybdate by adding ammonium sulphide to said mixture, the conversion being effected in the presence of a compound having a cation capable of combining with sulphur to produce an insoluble sulphide and with so much of the ammonium sulphide that no substantial quantity of ammonium sulfo-molybdate is formed, separating the ammonium sulfo-molybdate from the reaction mixture and adding thereto hydrochloric acid to precipitate molybdcic acid therefrom.

15. In the recovery of molybdenum from a material comprising molybdenum and at least one metal selected from the group consisting of magnesium, zinc and chromium, the steps which comprise subjecting the said material to a treatment with a gas capable of liberating free oxygen at a temperature ranging from 400° to 500° C., then converting the molybdenum oxides thus formed into soluble ammonium molybdate by treating the resulting mixture with a solution containing ammonia and so much ammonium sulphide in the presence of so much of a compound having a cation capable of forming an insoluble sulphide that no substantial quantity of ammonium sulfo-molybdate remains after the conversion.

20. The process of recovering molybdenum from a mixture containing it and at least one metal selected from the class consisting of zinc, magnesium and chromium which comprises treating the mixture with a gas capable of liberating free oxygen at a temperature ranging from 400° to 500° C. to effect a conversion of the metallic constituents of said mixture into the oxidic state, converting the oxides of molybdenum in said mixture into ammonium molybdate by adding ammonium sulphide to said mixture, the conversion being effected in the presence of a compound having a cation capable of combining with sulphur to produce an insoluble sulphide and with so much of the ammonium sulphide that no substantial quantity of ammonium sulfo-molybdate is formed, separating the ammonium sulfo-molybdate from the reaction mixture and adding thereto hydrochloric acid to precipitate molybdcic acid therefrom.

25. In the recovery of molybdenum from a spent catalyst employed in the destructive hydro-

genation of carbonaceous materials and which

30. consists of about molecular proportions of molyb-

denum, zinc and magnesium in the form of

35. their compounds with at least one of the first

two elements of the sixth group of the periodic

40. system, the steps which comprise subjecting said

45. catalyst to careful roasting at from 460° to 480°

C. and treating the resulting mixture with a

50. gradual addition of a 10 per cent solution of

55. ammonium sulphide containing about 2 per cent

60. of free ammonia until the color changes from

65. light yellow to orange.

6. In the recovery of molybdenum from a

70. spent catalyst employed in the destructive hy-

75. drogenation of organic substances and which

80. consists of about 0.7 molecular proportion of

85. molybdenum and about 0.3 molecular proportion

90. of zinc in the form of their compounds with at

95. least one of the first two elements of the sixth

100. group of the periodic system, the steps which

105. comprise subjecting said catalyst to careful

110. roasting at from 460° to 480° C. and treating

115. the resulting mixture with an ammoniacal liq-

120. uor obtained by mixing one part of 10 per cent

125. ammonium sulphide solution with about 0.4 part

130. of 10 per cent aqueous ammonia, using such an

135. amount of the said liquor that no substantial

140. quantity of ammonium sulfo-molybdate is

145. formed.

ERNST POKORNY. 135

7. In the recovery of molybdenum from a material comprising molybdenum and at least one metal selected from the group consisting of magnesium, zinc and chromium, the steps which comprise subjecting the said material to a treatment with a gas capable of liberating free oxygen at a temperature between 400 and 600° C., converting the molybdenum oxides thus formed into soluble